

Nov. 8, 1960

J. A. R. FAUCHER ET AL

2,959,281

FLOTATION OF NIOBUM-BEARING MINERALS

Filed Dec. 31, 1958

3 Sheets-Sheet 1



Fig. 1

INVENTORS  
J. A. Roland FAUCHER  
Silien DESSUREAUX

BY

*John R. Faucher*  
ATTORNEYS

Nov. 8, 1960

J. A. R. FAUCHER ET AL

2,959,281

FLOTATION OF NIOBIUM-BEARING MINERALS

Filed Dec. 31, 1958

3 Sheets-Sheet 2



Fig. 2

INVENTORS  
J.A. Roland FAUCHER  
Silien DESSUREAUX

BY

ATTORNEYS

Nov. 8, 1960

J. A. R. FAUCHER ET AL.

2,959,281

## FLOTATION OF NIOBIUM-BEARING MINERALS

Filed Dec. 31, 1958

3 Sheets-Sheet 3



Fig. 3

INVENTORS  
J.A. Roland FAUCHER  
Silien DESSUREAUX

BY

**ATTORNEYS**

1

2,959,281

## FLOTATION OF NIOBUM-BEARING MINERALS

J. A. Roland Faucher and Silien Dessaureaux, Montreal, Quebec, Canada, assignors to Technical Managers Inc., West, Montreal, Quebec, Canada

Filed Dec. 31, 1958, Ser. No. 784,391

15 Claims. (Cl. 209—12)

This invention relates to the beneficiation by froth flotation of the niobium-bearing minerals (niobates) from their ores. More particularly, it is concerned with the separation of niobium-bearing minerals, such as pyrochlore, perovskite, niocalite, betafite and the like, from the other constituents of their ores.

The typical problems involved as well as their solutions are found in the production of pyrochlore concentrates.

Up to a relatively recent date, niobium, also known as columbium, was considered as a rather rare constituent of the earth's crust. This has prevented a wide-spread use of the element which was rather costly. The discovery of large deposits of pyrochlore-bearing rocks in various parts of the world will lead the industry into a larger use of niobium since there is no more risk of a lack of production.

Niobium ores being much more abundant than anticipated will cause the price of the element to decrease and this also will promote further usage. There is no doubt that pyrochlore ore will eventually become the major source of niobium.

The main usage of niobium is in the manufacture of high-temperature alloys which become more and more essential in this age of jet propulsion and rocket missiles. Niobium in addition, stands a good chance of being used in atomic piles on account of its high corrosion and temperature resistance, coupled with good structural behaviour.

In commercial practice, the use of niobium oxides, ferro-niobium and niobium metal has become increasingly important and, accordingly, the demand for high grade concentrates from which they may be recovered has steadily increased. Unfortunately, while there are large natural deposits of niobium minerals, the grade of these ores in most cases is not sufficiently high to make recovery of niobium therefrom commercially feasible, and no process has been available for readily and effectively producing concentrates of niobium-bearing minerals sufficiently rich in  $Nb_2O_5$  to be commercial.

Particularly is this true of most pyrochlore deposits within Canada and elsewhere in the world. Therefore, while the process is not limited thereto, the invention will be illustrated by its application to niobium ores and pyrochlores in particular.

Natural deposits of niobium-bearing minerals are usually ores containing, in addition to the niobium-bearing minerals, such as pyrochlore, perovskite, niocalite, betafite and the like, a mixed gangue composed of carbonates, phosphates, mica, iron minerals, silicates, etc. Such a mixed gangue may be comprised, for instance, of calcite, apatite, biotite, magnetite and pyroxene, and also metallic sulphides such as prite, pyrrhotite, sphalerite and galena. The proportions of the various constituents of gangue may, of course, vary considerably depending on the origin of the ore. Ordinarily, this mixed gangue content must be reduced to produce a concentrate meeting commercial standards, for example, to be used as raw

2

material for the production of niobium metal or salts, and ferro-niobium.

It is, therefore, the principal object of the present invention to provide a sequence of operations and a process by which a concentrate satisfactorily high in  $Nb_2O_5$  content can be obtained. It is also an object to provide a process whereby this is accomplished in an economical manner and with good recovery. It is a further object to provide suitable reagents for use in this process, which 10 reagents are simple in use, readily obtainable and effective in operation.

It is with the increase in the  $Nb_2O_5$  assay that the present invention is primarily concerned. This problem has been extremely difficult to solve, mainly because the 15 niobium-bearing minerals, with which this invention is concerned, have been considered either as non-floatable or as having a very low floatability index. Moreover, the problem was complicated by the absence of knowledge of a selective depressant for the niobium-bearing minerals 20 when attempts were made to increase the  $Nb_2O_5$  of the ore by removing by flotation some of the gangue constituents.

In accordance with the main characteristic of the present invention, it has been found that the niobium bearing minerals can be floated with a good separation from the remaining gangue constituents by means of a cationic promoter of the amine type, and a selective activator for the niobium bearing minerals containing a source of free ions selected from the group consisting of fluoride and 30 fluosilicate ions, the froth flotation being carried out in an acidic circuit. Preferably the cationic promoter is selected from mono-amine and di-amine acetates and heterocyclic organic amines. The source of fluoride or fluosilicate ions acts as an activator and/or anti-depressant 35 for neutralizing the effect of the depressants used in the process prior to the flotation of the niobium bearing minerals.

In accordance with the present invention, separation of the niobium-bearing minerals from their gangue is 40 accomplished either by conditioning the feed with a depressant for the niobium-bearing minerals, floating off the bulk of the gangue in single or stage operations, recovering the magnetic-iron minerals and the micas if desired, and conditioning the remaining ore with the above 45 noted novel reagent combination that promote an effective and selective flotation of the niobium minerals, more particularly the pyrochlore; or by conditioning the feed for floating off the niobium-bearing minerals along with the bulk of the oxides and silicates, rejecting as tailings 50 the bulk of the carbonate content, recovering from this bulk concentrate the micas and magnetic minerals if desired, and submitting the residual concentrate to the selective niobium minerals flotation.

The process is illustrated by the accompanying drawings in which:

Figure 1 is a flow sheet delineating the principal steps involved in the process of the present invention, for treating ore high in carbonate content, the bulk of this carbonate gangue being floated off as a preliminary concentration step;

Figure 2 is a flow sheet delineating the principal steps involved in the process for treating ore high in silicate content; and

Figure 3 is a flow sheet delineating the principal steps 65 involved in the process for treating ore high in carbonate content, the bulk of this carbonate gangue being rejected as a tailing when floating off a bulk silicate-oxide concentrate, as a preliminary concentration step.

Although not a part of the present invention, if the 70 feed is a natural ore, a careful preparation before flotation is usually found advisable. As shown in the drawings, this comprises grinding and classification or other-

wise reducing the ore to a suitable size for froth flotation feed, normally to about minus 35 mesh and preferably minus 50 or minus 60 mesh. Any combination of crushing, grinding and classification steps may be used.

If the ore has more than about 10% by weight of carbonates and phosphates, the procedure outlined in Figure 1 or 3 will be preferably followed. If the ore has less than about 10% by weight of carbonates and phosphates and has a high silicate content, the procedure outlined in Figure 2 is preferred. In accordance with the procedure illustrated by Figure 1, after the feed has been prepared as outlined above, the ground pulp is conditioned with niobium minerals depressants and a calcite-apatite promoter. This conditioning step is carried out at high solids although it may be done at flotation density if so desired. The niobium mineral depressant may be either caustic starch or an alkali silicate. Such a depressant is necessary because some or part of the niobium minerals react the same as calcite and apatite to most anionic type promoters. It is necessary, therefore, that a depressant be found of one constituent or the other.

The caustic starch actually comprises a mixture of an alkali such as sodium hydroxide and starch. Preferably, it is fed as a solution containing about 5-10% dissolved solids. The alkali-starch ratio may vary from as little as about 1:3 to as high as 3:1.

A sufficient amount should be used to produce depression of the niobium-minerals, the solution being added and conditioned with the pulp for sufficient time to ensure thorough dissemination.

It has been found also that successful results are readily obtained using a water-soluble silicate as niobium-mineral depressant. Usually, the amount of silicate required is about 1 to 3 pounds per ton of feed.

Other depressants may be used but these two groups have been found to be the most effective.

The time of conditioning will depend on the characteristics of the particular ore being treated, usually about 5 minutes are sufficient.

Either concurrently with or subsequently to this operation, an anionic promoter for calcite and apatite is added. This promoter may be one of several types; a fatty acid such as oleic, stearic, palmitic, fish-oil fatty acids, cocoanut oil fatty acid, and the like, or soaps thereof, as well as the various commercial mixtures thereof and naphthenic acids or their soaps. Such naturally occurring mixtures of fatty and resin acids such as tallow or residue such as cotton-seed-foot oil or their soaps are also satisfactory, as well as sulphonated reagents such as sulphonated higher aliphatic alcohols, sulphonated fatty acids. Sulphonated petroleum hydrocarbons may also be used per se or in conjunction with another promoter; cotton-seed-foot oil has been found to give excellent results in conjunction with a petroleum sulphonate and since it is readily available and inexpensive, is perhaps preferable.

In general, the amount of promoter required is about 1.5 to 3.0 lb./ton. Excessive amounts over that should necessarily be avoided as tending to overcome the effect of niobium minerals depressant and to increase the losses in the subsequent flotation.

If conditioning was at high solids the pulp is first reduced to flotation density of from 15-25% solids before being subjected to flotation, which is carried until the calcite and apatite removal is apparently complete.

The addition of a small quantity of frother to the flotation cell is usually beneficial during this operation. Stage addition of reagents to the flotation circuit is often useful to assure complete removal of the calcite and the apatite.

The condition and flotation procedures are usually advantageously repeated in sustained commercial operations taking off a second calcite-apatite concentrate or middling product, to assure the most economical complete removal of these minerals.

These calcite-apatite concentrates are usually combined and subjected to a cleaner and recleaner flotation. A small addition of niobium minerals depressant, about 1.0 lb./ton is usually beneficial in these cleaning operations. As the object of these cleanings is to reduce the niobium losses encountered in the bulk flotation of calcite and apatite, the cleaner tails, which are enriched in  $\text{Nb}_2\text{O}_5$  are recycled to the original flotation feed, or to any other point in the circuit which might be found more advantageous, like the classification, the conditioning or the calcite-apatite flotation.

The tailing from this first step of concentration contains most of the  $\text{Nb}_2\text{O}_5$  (95%+) contained in the original feed, mixed with some minerals like mica, magnetite, diopside, etc.

This tailing could be treated to recover the mica and the magnetite, which are saleable products or could be fed directly to the niobium mineral flotation.

On account of their commercial by-product values, it is sound economically to recover at this stage the mica and the magnetite. These minerals can be recovered in that order, but the magnetite can be recovered first if desired.

To obtain the mica concentrate, the machine discharge or tailing from the calcite-apatite concentration is decanted or dewatered to remove the excess and the effect of the reagents used in the preceding flotation. It has been found unnecessary at this stage to use a scrubbing treatment to effect this reagent's removal.

This dewatering can be effected in a large pool classifier or in a thickener. The thickened pulp is then conditioned with a mica promoter which in this case is any good cationic promoter of the primary mono amine acetate type such as coco amine, soya amine and the like or of the diamine acetate type such as coco diamine or tallow diamine and the like. Amine 220, which is a trade name of Union Carbide and Carbon Corporation for 1-hydroxyethyl-2-heptadecenyl glyoxalidine, and "Aeromine" 2026, which is a trademark for an amine cationic flotation reagent of uncertain composition made by the American Cyanamid Co., have been found to give excellent results. In general the amount required is relatively small, about 0.4 lb./ton of flotation feed.

At the same time, the niobium mineral depressant is added. Caustic starch, added at the rate of 0.5 to about 1.5 lb./ton has given good results at this stage and was used preferably. A slight amount of frother, about 0.05 lb./ton added to the flotation cell is ordinarily helpful to carry this flotation. This mica flotation is a basic circuit in the presence of causticized starch, produces a selective separation of the pyrochlores from the mica, and is an important feature of this invention.

As in the case of the calcite-apatite flotation, cleaning of the mica concentrate with a small addition of niobium depressant (about 0.2 lb./ton of causticized starch), is advantageous to minimize the niobium losses carried over with the mica concentrate. The tailing from this cleaner operation is either returned at the head of the mica flotation, like at the decantation feed, or at such other point in the circuit that might be found more advantageous.

The machine discharge or tailing from the mica flotation could be fed to the magnetite recovery circuit, if the recovery of this iron concentrate is desired.

The circuit consists of any appropriate drum type or belt type low or medium intensity wet magnetic concentrator. The magnetite, which is highly magnetic is attracted by the magnetic field, while the rest of the ore is unaffected, making the separation possible.

One or two cleanings of the magnetite concentrate in similar type magnetic separators is advisable to raise the grade of the magnetite concentrate to saleable grade and to liberate the non-magnetic ore particles mechanically trapped between the magnetite grains during the separation process. These cleaner tails are again returned to

the head of this circuit or by-passed directly with the magnetite tailings to the following operation stage.

At this point, one has reached the stage where the niobium-bearing minerals (the pyrochlore) can be directly floated off into a high grade concentrate.

As stated previously, the feed to the pyrochlore flotation could be either the calcite-apatite flotation tailings, by-passing the mica and the magnetite removals, or the tailings from the mica flotation, or the tailings from the magnetic separation.

If the mica flotation is by-passed, the pyrochlore flotation can proceed with the addition of a specific mica depressant, like one of the arabic gums such as guar gum, quartex and the like, a glue, starch or any other appropriate mica depressant fed at the rate of about 0.5 lb./ton. The mica flotation is delayed this way but not enough to produce a one pass clean separation of the pyrochlore from the mica, and three or four successive pyrochlore concentrate cleanings are required to bring out the optimum pyrochlore concentrate grade.

The pyrochlore flotation procedure is not modified whether the magnetic separation is performed or not. The tailing or reject from the previous concentration operation is decanted or dewatered to remove the effect and the excess of the reagents already used in previous operations.

This thickened pulp is then conditioned for the niobium minerals flotation. Heavy solid (50% solid) conditioning, though preferable, is not absolutely required, and dilution of the pulp to flotation density, about 25% solid can be effected before or after the conditioning.

Where conditioning at high solids, or even conditioning prior to flotation cannot be employed, it is possible to add the reagents directly to the flotation cell. This practice is undesirable and should be avoided if possible, since it requires more reagent and/or longer treatment in the cells, and even then is not as satisfactory. It is also an advantage of the present invention that it permits the use of readily-available cationic-type promoters such as described in the mica flotation.

The amount of promoter used will vary with the nature of the ore, the water conditions, i.e. temperature, acidity, hardness, etc., of the water and the average particle size mineral and content of the feed being treated. In general an amount ranging from 0.5 to 1.5 lbs./ton of ore treated is necessary. In some cases, a frother may be useful. Where a frother is desirable, any suitable type such as pine oil, cresylic acids and the commercial higher alcohol frothers may be used.

Of primary importance is also the use of the novel activator and selectivity-assisting agent for the pyrochlore minerals, of this invention. This activator may also act as an antidepressant to neutralize the depressing effect of the reagents used in the prior steps of the process described: such as causticized starch, sodium silicates or others. This activator should be an effective source of fluoride and/or fluosilicate ions. The particular source may be varied. The necessary ions may be provided, for example, per se or as a soluble salt thereof. Where the circuit itself is not normally acidic (pH lower than 7) it should be made so. This may be done by adding an acid such as HF,  $H_2SiF_6$ . It may also be done by adding a soluble fluosilicate such as that of sodium or potassium, since these salts have an acid reaction. Similarly, a combination of a mineral acid, sulfuric, hydrochloric or the like may be used with a soluble fluoride or acid fluoride such as those of sodium, potassium or ammonium.

As to the amount of activator used, the demand may be quite flexible. In general it will vary between 2 to 6 lbs./ton of feed.

Good results were obtained by adding about 2 lbs./ton in the initial conditioning or to the cells during the rougher flotation if preconditioning is not used, and small additions stage fed during flotation and cleaning.

The diluted conditioned pulp is then sent to the rougher

flotation circuit as is shown in Figure 1. An excellent separation of the pyrochlores from the rest of the ore is obtained. This rougher concentrate may be sent to a cleaner flotation, to further upgrade its  $Nb_2O_5$  assay.

5 The tailing from the cleaner circuit can be recycled to the feed of the rougher flotation, or at any particular point found most advantageous.

If the ore contains a substantial proportion of metallic sulfides, particularly pyrite, it is possible in accordance with the present invention to collect a pyrite concentrate without affecting the subsequent pyrochlore flotation. The feed for the pyrite flotation may be either the calcite-apatite flotation tailings, or the tailings from the magnetic separation.

15 The tailings are conditioned for about 5 minutes with a xanthate, in a basic, neutral or acidified circuit. The pyrite is floated and the tailing constitutes the feed for the pyrochlore flotation described hereinabove.

When the ore to be treated contains only a small proportion of carbonate and phosphates (about 10% and less) and has a high silicate content, the calcite-apatite flotation may be by-passed as shown in Figure 2.

20 The prepared feed can be fed directly to the mica flotation and thence to the magnetic separation and the resultant tailings subjected to the pyrochlore flotation.

25 It is also possible to subject the prepared feed only to the pyrochlore flotation, by-passing both the mica flotation and the magnetic flotation; in this case the pyrochlore flotation will be effected with the addition of a specific mica depressant such as guar as described hereinabove with respect to Figure 1.

30 In accordance with the procedure illustrated in Figure 3, the preliminary concentration step consists in floating off the bulk of the silicate and oxide content of the ore, along with the niobium-bearing minerals, and discarding most of the carbonate and phosphate content as flotation tailings. This bulk silicate-oxide concentrate is similar in composition to the product previously referred to as "The tailing from the first step of concentration, containing 35 most of the  $Nb_2O_5$  contained in the original feed, mixed with some minerals like mica, magnetite, diopside, etc.," and is processed to obtain the final niobium concentrate, the same way as described in discussing the process illustrated in Figure 1, for mica, magnetite and 40 sulfides, optional removal, and niobium minerals flotation.

45 After the feed has been adequately prepared, the ground pulp is conditioned for about 2 minutes with a cationic collector or promoter of the same family referred to in the mica and niobium-mineral flotations. This conditioning is usually performed at high solids ( $\pm 50\%$  solids) although it may be done at flotation density if so desired.

50 Usually, the amount of collector required is about 1 to 3 pounds per ton of feed.

If conditioning was at high solids, the pulp is first reduced to flotation density of from 15-25% solids before being subjected to flotation, which is carried until the silicates and oxide removal is apparently complete.

55 60 Staged addition of reagents to the flotation circuit is often useful; conditioning and flotation procedures can be advantageously repeated in sustained commercial operations taking off a second silicate-oxide concentrate, to assure the most economical complete removal of these minerals, particularly the pyrochlores.

65 The residue from this flotation is the calcite-apatite concentrate, while the concentrate contains most of the niobium minerals and is further processed for niobium recovery the same way as the residue from the calcite-apatite flotation was treated in the discussion of the process illustrated by Figures 1 and 2.

70 75 This invention may be illustrated in conjunction with the following examples, which are illustrative only and not by way of limitation. All parts are by weight unless otherwise noted.

## EXAMPLE I

## Calcite-apatite flotation—Mica flotation—Magnetic separation—Pyrochlore flotation

A sample of ore from the Oka district, Province of Quebec, Canada, comprising pyrochlore with a gangue containing mainly calcite, apatite, mica, pyroxene, magnetite and pyrite was given a preliminary treatment by crushing and grinding to minus 65 mesh.

A pulp of the ore comprising about 50% solids in water was conditioned for 5 minutes with 0.8 lbs./ton of oleic acid, 1.2 lbs./ton of Petronate L (a trademark of L. Sonneborn Sons Inc., New York City for a salt of a petroleum sulfonic acid), and 2 lbs./ton of water glass (sodium silicate).

This conditioned pulp was then reduced to about 20% solids, the calcite-apatite concentrate floated, and the concentrate was cleaned with 1 lb./ton of sodium silicate. The cleaner tails were combined with the flotation tails.

These tailings were dewatered to about 60% solids and conditioned 5 minutes for mica flotation with 1.0 lb./ton of causticized starch having an alkali-starch ratio of 1 to 3 and 0.5 lb./ton of Amine 220. The conditioned pulp was then diluted to about 20% solids, and the mica concentrate floated off. This concentrate was cleaned twice with the addition of 1.0 lb./ton of causticized starch to the cleaner cells.

The cleaner tails were combined with the flotation tails and treated by magnetic concentration to recover a magnetite concentrate, which was given one cleaning pass.

The cleaner tails and the tailings from the magnetic concentration were dewatered to about 60% solid and conditioned 6 minutes with 4.0 lb./ton of HF, and 0.5 lb./ton of "Aeromine" 2026. The conditioned pulp was reduced to about 20% solid and the pyrochlore concentrate floated off. This concentrate was given two cleanings with the addition of 0.5 lb./ton of HF at each cleaning.

The two cleaner tails were combined for assaying.

The results obtained are shown in the following Table I.

Table I

| Products                      | Percent Weight | Percent Nb <sub>2</sub> O <sub>5</sub> | Nb <sub>2</sub> O <sub>5</sub> |                       |
|-------------------------------|----------------|----------------------------------------|--------------------------------|-----------------------|
|                               |                |                                        | Units                          | Distribution, Percent |
| Feed                          | 100.0          | 0.55                                   |                                |                       |
| Calcite - Apatite Concentrate | 73.0           | 0.06                                   | 4.4                            | 8.1                   |
| Mica Concentrate              | 5.7            | .70                                    | 4.0                            | 7.3                   |
| Magnetic Concentrate          | 2.7            | 0.15                                   | .4                             | .7                    |
| Pyrochlore Concentrate        | 1.2            | 29.5                                   | 35.4                           | 64.6                  |
| Pyrochlore Cleaner tails      | 2.2            | 1.92                                   | 4.2                            | 7.6                   |
| Tailings                      | 15.2           | .42                                    | 6.4                            | 11.7                  |

These results indicate that this process permits an economical recovery of a high grade pyrochlore concentrate, containing 29.5% Nb<sub>2</sub>O<sub>5</sub> and representing an estimated overall recovery of better than 70%. It also permits the production of mica and magnetite concentrates as commercial by-products, and this with acceptable Nb<sub>2</sub>O<sub>5</sub> losses.

## EXAMPLE II

The whole ore was treated as in the Example I to remove a calcite-apatite concentrate, followed by magnetic concentration to remove a magnetite concentrate, and then the dewatered combined tailings and cleaner tails were conditioned directly for the pyrochlore flotation, bypassing the mica flotation.

The reagents used in the pyrochlore flotation conditioning were HF at 3 lbs./ton, "Aeromine" 2026 at 0.8 lb./ton, and guar at 0.5 lb./ton to favor the mica depression.

The pyrochlore concentrate was cleaned three times and the cleaner tails combined for assaying.

This procedure gave the following results:

5

Table II

|    | Products                    | Percent Weight | Analysis, Percent Nb <sub>2</sub> O <sub>5</sub> | Percent Recovery Nb <sub>2</sub> O <sub>5</sub> |
|----|-----------------------------|----------------|--------------------------------------------------|-------------------------------------------------|
| 10 | Calcite-apatite concentrate | 73.0           | .04                                              | 5.1                                             |
|    | Magnetite concentrate       | 2.8            | .14                                              | .7                                              |
|    | Pyrochlore concentrate      | 1.1            | 36.8                                             | 71.5                                            |
|    | Cleaner tails               | 2.3            | 1.65                                             | 6.7                                             |
|    | Tailings                    | 20.8           | .46                                              | 15.9                                            |
|    | Feed (Calculated)           | 100.0          | .57                                              | 99.9                                            |

15

## EXAMPLE III

The whole ore was treated as in Example I to remove a calcite-apatite concentrate and the dewatered tailings from this flotation were conditioned directly for the pyrochlore flotation, bypassing the iron and mica removals.

20

The reagents used in the pyrochlore flotation conditioning were HF at 5 lbs./ton, Amine 220 at 0.6 lbs./ton, and guar gum at 0.4 lbs./ton to favor the mica depression.

25

The pyrochlore concentrate was cleaned twice only with the addition of 0.2 lbs./ton of guar gum and 0.4 lbs./ton of Amine 220 to the cleaner flotation, and the cleaner tails combined for assaying.

30

The results obtained through this procedure are tabulated in Table III.

Table III

|    | Products                    | Percent Weight | Percent Nb <sub>2</sub> O <sub>5</sub> | Distribution, Percent Nb <sub>2</sub> O <sub>5</sub> |
|----|-----------------------------|----------------|----------------------------------------|------------------------------------------------------|
| 35 | Calcite-apatite concentrate | 70.1           | 0.06                                   | 9.5                                                  |
|    | Pyrochlore concentrate      | 1.2            | 22.6                                   | 61.8                                                 |
|    | Cleaner tails               | 1.8            | 1.95                                   | 8.0                                                  |
|    | Tailings                    | 26.9           | 0.34                                   | 20.7                                                 |
|    | Feed (calculated)           | 100.0          | 0.44                                   | 100.0                                                |

40

These results indicate clearly the possibility of a successful selective concentration of the pyrochlore directly after the removal of the carbonaceous constituents of the ore.

45

The grade of 22.6% Nb<sub>2</sub>O<sub>5</sub> can be improved with successive cleaning operations.

## EXAMPLE IV

The whole ore was treated as in Example I to remove a calcite-apatite concentrate, followed by magnetic concentration to remove a magnetite concentrate. The tailings from this concentration were conditioned for 5 minutes with a xanthate (0.5 lbs./ton of Z-6, an amyloxanthate from Dow Chemical), and 1.0 lbs./ton of sulfuric acid, for the removal of metallic sulfides, particularly pyrite. The dewatered tailings from this flotation were then conditioned with the same reagents, as used in Example II; the pyrochlore concentrate was cleaned only once. This procedure gave the following results.

60

Table IV

|    | Products                    | Percent Weight | Percent Nb <sub>2</sub> O <sub>5</sub> | Percent Nb <sub>2</sub> O <sub>5</sub> Recovery |
|----|-----------------------------|----------------|----------------------------------------|-------------------------------------------------|
| 65 | Calcite-apatite concentrate | 66.6           | 0.02                                   | 3.2                                             |
|    | Pyrite concentrate          | 2.8            | 0.20                                   | 1.3                                             |
|    | Magnetite concentrate       | 2.6            | 0.15                                   | 1.0                                             |
|    | Tailings 2                  | 19.0           | 0.23                                   | 10.6                                            |
|    | Cleaner Tails               | 6.8            | 0.65                                   | 10.7                                            |
|    | Pyrochlore concentrate      | 2.24           | 13.5                                   | 73.2                                            |
|    | Feed (calculated)           | 100.04         | 0.41                                   | 100.0                                           |
|    |                             | 100.0          | 0.41                                   | 100.0                                           |

These results are indicative that very good concentration of the pyrochlore can be effected, after metallic sulfides recovery, if such a recovery is found desirable.

75

More cleanings of the pyrochlore concentrate would be necessary to up-grade this concentrate to above 20%  $\text{Nb}_2\text{O}_5$ .

#### EXAMPLE V

A pulp of the ore comprising about 50% solids in water was conditioned for 2 minutes with 1.0 lbs./ton of Aeromine 2026 and 0.5 lbs./ton of Amine 220. This conditioned pulp was then reduced to about 25% solids, and the silicate and oxide minerals, together with the niobium minerals floated off.

Staged addition of collectors to the flotation cell at the rate of 0.3 lbs./ton of each of the collectors: (Aeromine 2026 and Amine 220) was made to ascertain the complete collection of the niobium minerals.

The tailings from this flotation contained mostly the calcite and the apatite and was rejected as a calcite-apatite residue.

The concentrate so obtained contained most of the niobium minerals and was further treated for the optimum concentration of these minerals.

This concentrate was dewatered to about 50% solids and submitted to mica flotation the same way as described in Example I.

The mica-flotation tailing was then submitted directly to the selective pyrochlore flotation as also described in Example I.

The results obtained by this procedure were as follows:

Table V

| Products                      | Percent Weight | Percent $\text{Nb}_2\text{O}_5$ | Percent $\text{Nb}_2\text{O}_5$ Recovery |
|-------------------------------|----------------|---------------------------------|------------------------------------------|
| Feed.....                     | 100.0          | 0.51                            | 100.0                                    |
| Calcite-apatite residue.....  | 56.3           | 0.03                            | 3.3                                      |
| Mica concentrate.....         | 11.7           | 0.50                            | 11.4                                     |
| Pyrochlore Conc.....          | 1.1            | 30.50                           | 66.0                                     |
| Pyrochlore Cleaner Tails..... | 2.2            | 1.60                            | 6.9                                      |
| Tailings.....                 | 28.7           | 0.22                            | 12.4                                     |

These results indicate that this process permits an economical recovery of a high grade pyrochlore concentrate, containing 30.5%  $\text{Nb}_2\text{O}_5$  and representing an estimated overall recovery of better than 71%.

#### EXAMPLE VI

The whole ore was treated as in Example V, the cationic collectors being added at the rate of 0.6 lbs./ton of Amine 220 and 1.5 lbs./ton of Aeromine 2026. This combination of reagents gave better frothing characteristics to the flotation.

The mica was removed and the pyrochlore flotation proceeded with as in Example V.

The results obtained are shown in the following table:

Table VI

| Products                    | Percent Weight | Percent $\text{Nb}_2\text{O}_5$ | Distribution, Percent $\text{Nb}_2\text{O}_5$ |
|-----------------------------|----------------|---------------------------------|-----------------------------------------------|
| Feed.....                   | 100.0          | 0.55                            | 100.0                                         |
| Cal-apatite Residue.....    | 61.2           | 0.03                            | 3.3                                           |
| Mica Concentrate.....       | 11.1           | 0.55                            | 11.1                                          |
| Pyrochlore Concentrate..... | 1.1            | 34.3                            | 68.3                                          |
| Pyrochlore Cl-Tails.....    | 2.0            | 1.70                            | 6.2                                           |
| Tailings.....               | 24.6           | 0.25                            | 11.1                                          |

These results indicate an overall estimated recovery of about 72% in a concentrate containing 34.3%  $\text{Nb}_2\text{O}_5$ . This method of processing can then produce a successful selective concentration of the pyrochlore.

From these results it will be seen that not only is the process of the present invention adapted to produce satisfactory high grade concentrates, with high recovery, but it is well adapted for continuous operation.

We claim:

1. A process for beneficiating a mixture of minerals comprising a low concentration of oxidized niobium min-

erals dispersed in a large amount of gangue, said mixture being ground to particle sizes suitable for froth flotation feed, which comprises forming an aqueous pulp of said mixture, subjecting said aqueous pulp to froth flotation in the presence of a cationic promoter of the amine type and a selective activator for the niobium-bearing mineral selected from the group consisting of fluoride and fluosilicate ions, and collecting the resultant niobium-rich flotation concentrate, separately from the niobium-poor flotation tailing.

5 2. A process as claimed in claim 1, wherein the aqueous pulp subjected to froth flotation is at a pH lower than 7.

3. A process as claimed in claim 1, wherein a frother is added to the aqueous pulp.

4. A process as claimed in claim 3, wherein said frother is selected from pine oil, cresylic acid and higher alcohols.

5. A process as claimed in claim 1, wherein said cationic promoter is selected from monoamine and diamine acetate and heterocyclic organic amines.

6. A process as claimed in claim 1, wherein said gangue includes mica and wherein a mica depressant is added to the aqueous pulp subjected to froth flotation.

25 7. A process as claimed in claim 6, wherein said mica depressant is selected from gum arabic, gum guar, glues and starch.

8. A process as claimed in claim 1, wherein said gangue includes a substantial amount of calcite and apatite, including the preliminary steps of subjecting the aqueous pulp to flotation in the presence of an anionic promoter selected from the group consisting of the higher fatty acids, resin acids, naphthenic acids, mixtures thereof, their soaps, sulphonated petroleum hydrocarbons and higher aliphatic alcohols, and a depressant selected from the group consisting of caustic starch and an alkali silicate, collecting the resultant flotation concentrate as a calcite-apatite concentrate substantially from niobium bearing minerals, separately collecting the residual tailing as a concentrate of niobium-bearing mineral substantially free from apatite and calcite, and using said last named concentrate as the feed for the froth flotation of the niobium-bearing minerals.

9. A process as claimed in claim 8, wherein the caustic starch is a mixture of starch and an alkali, the alkali-starch ratio being between about 1:3 and 3:1.

10. A process as claimed in claim 1, wherein said gangue includes a substantial amount of mica, including the preliminary steps of subjecting the aqueous pulp to froth flotation in the presence of a cationic promoter of the amine type and of caustic starch as a niobium mineral depressant, collecting the resulting flotation concentrate as a mica concentrate substantially free from niobium-bearing minerals and separately collecting the residual tailing as a concentrate of niobium-bearing minerals substantially free from mica, and using said last named concentrate as the feed for the froth flotation of the niobium-bearing minerals.

11. A process as claimed in claim 1, wherein said gangue includes a substantial amount of magnetic minerals, the preliminary steps of subjecting the aqueous pulp to a magnetic separation, collecting a concentrate having a high iron assay and separately collecting the residual tailing as a concentrate of niobium-bearing minerals substantially free of magnetic minerals, and using said tailing as the feed for the froth flotation of the niobium-bearing minerals.

12. A method of beneficiating ores of niobium-bearing minerals, more particularly pyrochlores, containing excessive amounts of gangue material, which comprises the steps of reducing the ore to suitable size for flotation feed, conditioning the pulp with an effective amount of an anionic type promoter selected from the group consisting of the higher aliphatic fatty acids, resin acids, naphthenic acids, cotton-seed-foot-oil, oleic acid, mix-

tures thereof and their soaps, sulphonated petroleum hydrocarbons, higher aliphatic alcohols, and mixtures thereof, and an effective amount of niobium-bearing mineral depressant selected from causticized starch and alkali silicates, subjecting the conditioned pulp to froth flotation to float substantially all the carbonate and phosphorus bearing minerals therefrom, collecting and dewatering the resultant tailings, conditioning an aqueous pulp of these tailings with an effective amount of a substance selected from caustic starch and alkali silicates and with a cationic type promoter selected from primary mono- and di-amine acetates, subjecting the conditioned pulp to froth flotation to remove a mica concentrate, collecting the resultant tailings and subjecting them to magnetic separation to collect a magnetite concentrate, collecting and dewatering the resultant tailings, conditioning an aqueous acidic pulp of these tailings with an effective amount of cationic promoter for the niobium-bearing minerals selected from the same group from which the mica flotation promoter was selected and an effective amount of activator selected from the group consisting of fluoride and fluosilicate ions, subjecting the conditioned pulp to froth flotation, and collecting the resultant flotation concentrate as a high grade niobium concentrate.

13. A process as claimed in claim 1, wherein said gangue includes a substantial amount of calcite and apatite, including the preliminary steps of subjecting the aqueous pulp to flotation in the presence of a cationic promoter selected from the group consisting of cationic promoters of the primary mono amine acetate type, of the di-amine acetate type and of the heterocyclic amine type, collecting the resultant flotation concentrate as a niobium-bearing mineral, silicate and oxide concentrate substantially free from calcite and apatite, and using said last named concentrate as the feed for the froth flotation of the niobium-bearing minerals.

14. A method of beneficiating ores of niobium-bearing minerals, more particularly pyrochlores, containing an excess amount of gangue material, which comprises the steps of reducing the ores to suitable size for flotation feed, conditioning the pulp with an effective amount of cationic promoter of the amine type, subjecting the con-

ditioned pulp to froth flotation to float a concentrate containing substantially all the niobium-bearing minerals together with silicates and oxides and substantially free from all the carbonate and phosphorus bearing minerals, 5 collecting said concentrate, conditioning an aqueous pulp of said concentrate with an effective amount of a substance selected from caustic starch and an alkali silicate and with a cationic promoter selected from primary mono and di-amine acetates and heterocyclic organic amines, subjecting the conditioned pulp to froth flotation to remove a mica concentrate, collecting the resultant tailings and subjecting them to magnetic separation to collect a magnetite concentrate, collecting and dewatering the resultant tailings, conditioning an aqueous acidic 10 pulp of these tailings with an effective amount of cationic promoter for the niobium-bearing minerals selected from the same group from which the mica flotation promoter was selected and an effective amount of an activator selected from the group consisting of fluoride and fluosilicate ions, subjecting the conditioned pulp to froth flotation, and collecting the resultant flotation concentrate as a high grade niobium concentrate.

15. A process as claimed in claim 1, wherein said gangue includes a substantial amount of metallic sulphides, including the preliminary steps of subjecting the aqueous pulp to froth flotation in the presence of a promoter of the xanthate type, collecting the resultant flotation concentrate as a metallic sulphide concentrate essentially free from niobium-bearing minerals and separately 20 collecting the residual tailings as a concentrate of niobium-bearing minerals substantially free from metallic sulphides, and using said last named concentrate as a feed for the froth flotation of the niobium-bearing minerals.

35 **References Cited in the file of this patent**  
**UNITED STATES PATENTS**

2,297,689 O'Meara ----- Oct. 6, 1942  
 2,875,896 Last et al. ----- Mar. 3, 1952

40 **OTHER REFERENCES**

Taggart "Handbook of Mineral Dressing," 1945, sec. 12, pp. 17, 24 and 44.

UNITED STATES PATENT OFFICE  
CERTIFICATION OF CORRECTION

Patent No. 2,959,281

November 8, 1960

J. A. Roland Faucher et al.

It is hereby certified that error appears in the above numbered patent requiring correction and that the said Letters Patent should read as corrected below.

In the grant (only), line 1, name of first inventor, for J. A. Roland Fucher" read -- J. A. Roland Faucher --; in the printed specification, column 4, line 10, after "like" insert -- to --; line 32, for "thise" read -- this --; line 49, for "is" read -- in --; column 10, line 38, for "from", first occurrence, read -- free --; line 39, for "separaely" read -- separately --.

Signed and sealed this 2nd day of May 1961.

(SEAL)

Attest:

ERNEST W. SWIDER  
Attesting Officer

DAVID L. LADD  
Commissioner of Patents